

# UNITED STATES PATENT OFFICE.

LINWOOD T. RICHARDSON, OF MILWAUKEE, WISCONSIN, AND ELWOOD A. RICHARDSON,  
OF CLEVELAND, OHIO.

## ALLOY.

1,317,592.

Specification of Letters Patent. Patented Sept. 30, 1919.

No Drawing.

Application filed June 3, 1918. Serial No. 237,904.

*To all whom it may concern:*

Be it known that we, LINWOOD T. RICHARDSON, a citizen of the United States, and ELWOOD A. RICHARDSON, a citizen of the United States, residing, respectively, at Milwaukee, county of Milwaukee, State of Wisconsin, and at Cleveland, county of Cuyahoga, State of Ohio, have invented certain new and useful Improvements in Alloys; and we do hereby declare the following to be a full, clear, and exact description of the invention, such as will enable others skilled in the art to which it appertains to make and use the same.

Our invention relates to ferrous alloys, and has for its general object the production of an improved rust or corrosion-resisting ferrous alloy.

Iron, in any of its well known commercial forms, oxidizes or rusts more or less easily when exposed to the atmosphere. While many expedients and agencies have heretofore been employed or suggested for preventing or minimizing this natural tendency of iron to oxidize, as far as we know, the beneficial effects of certain metallic substances in preventing or minimizing the natural tendency of iron in its usual commercial forms to rust have not been recognized. We have discovered that certain metals exercise in combination a very beneficial effect in minimizing the rusting or corrosion of iron when these metals are present therein in certain predetermined quantities. Thus, we have found that copper and manganese, when added in certain percentages to iron, produce a ferrous alloy having rust-resisting characteristics which are not possessed by iron without such additions of copper and manganese. The corrosion of the iron is lessened by the addition of either copper or manganese, but we have discovered that the two metals acting together produce an effect greater than either alone. And we have further found that the manganese may be in whole or in part replaced by chromium in which event the combined effect of the copper and chromium, or copper, manganese and chromium, is to minimize and materially reduce the natural tendency of the iron to rust, as compared with iron in which such modifying agents are not present within the percentages contemplated by our present invention.

The present invention involves the addition to or alloying with iron, in any of its usual commercial forms, of certain relatively small quantities of two or more metallic modifying agents, whose combined effect upon the iron is to increase or improve its rust-resisting properties. The beneficial effect resulting from the addition of two or more such modifying agents to iron is due to the combined action of the agents. Thus, while any one agent acting alone might improve the rust-resisting properties of iron, we have found that the combined action of two or more of the modifying agents produces a more pronounced improvement in the rust-resisting properties of iron than does any one agent when used alone.

The metallic modifying agents which we add to iron to improve or ameliorate its rust-resisting properties by their combined action may be divided into two classes, to wit, a major modifying agent and a minor modifying agent or agents. The major modifying agent is that which if alone added to the iron would produce the most marked improvement in the rust-resisting properties thereof, while the minor modifying agents are those which if alone added to the iron would produce some improvement in the rust resisting properties thereof, but not as great an improvement as the major modifying agent acting alone. And further, in accordance with the principles of our present invention, the major modifying agent in combination with one or more minor modifying agents produce a more marked improvement in the rust-resisting properties of the iron than does any single modifying agent.

As the major modifying agent, we prefer to use copper, since we have found that, acting alone, copper produces the greatest improvement in the rust-resisting properties of iron. In carrying out our present invention, we use in combination with copper, one or more minor modifying agents whose combined effect with copper is to produce a greater improvement in the rust-resisting properties of the iron than is produced by copper alone, or by any one of the minor modifying agents alone. As such minor modifying agents we prefer to use either manganese or chromium, or manganese and chromium.

We have determined, in using copper alone as the modifying agent for improving the rust-resisting properties of iron, that little advantage results in using more than 5 about 2.0% of copper, and for most practical purposes the most satisfactory results are obtained by using from 1.5% to 2% of copper. With manganese alone, we have found that the decrease in corrosion or rusting of the 10 iron is little marked up to about 2% of manganese. There is, however, little practical advantage in using a greater percentage of manganese, because ferrous alloys containing more than about 2% of manganese are brittle and hard to work, as will 15 be more fully explained hereinafter.

In accordance with the principles of our present invention, the copper and manganese operate together to produce a more 20 pronounced improvement in the rust-resisting properties of iron than would either metal if alone alloyed with iron. We have determined that little improvement in its 25 rust-resisting properties results from the addition of copper to a ferrous alloy containing more than about 1% of manganese, or from the addition of more than 2% of copper to a ferrous alloy of any manganese content. In general, we prefer to alloy with the 30 iron from about 1.0% to about 2% of copper and about 1% of manganese.

As we have hereinbefore mentioned, the manganese may be in whole or in part replaced by chromium. Generally speaking, 35 we have found it advisable to employ, in combination with copper, a slightly larger percentage of chromium than mentioned in the case of manganese. Thus, in using chromium alone, as the minor modifying agent, 40 we prefer to employ from about 1.5% to about 2% thereof. When both manganese and chromium are to be used in combination with from about 1% to about 2% of copper, we have found a combined manganese-chromium content of from about 1% to about 45 2% to give satisfactory results.

In the preceding paragraphs we have mentioned specific percentages which we have found to produce the most satisfactory results in improving the rust-resisting properties of ferrous alloys. We wish it to be understood, however, that we do not intend thereby to limit our invention to the employment of such specific percentages of the 50 modifying agents, since our invention in its broad aspect is capable of advantageous application without particular reference to the specific percentages mentioned. In its 55 broader aspect our invention thus contemplates the use of from about 1.5% to about 60 4% of a plurality of combined metallic modifying agents, each of which is present in quantities from about 0.5% to about 2%. The balance of the ferrous alloy is composed 65 principally of iron. And, of course, it will

be understood that the modifying agents are of such a character that they produce in combination a more pronounced improvement in the rust-resisting properties of the resulting ferrous alloy than would be produced by using any one of the modifying agents alone. 70

Alloys of iron and copper alone do not forge satisfactorily. When red hot such alloys are brittle and smash when struck with 75 a hammer. At low temperatures they can be forged by using extreme care, and by expending a great deal of energy. There appears to be a range of temperatures at which any particular copper-iron alloy cannot be 80 satisfactorily worked or forged at red heat. With increasing copper content this "red-short" or non-malleable temperature range occurs at a lower temperature and exists over a longer interval. For example, in the 85 case of one series of copper-iron alloys which we tested, we found that the iron with zero per cent. copper could be forged at all temperatures, with 0.25% copper the resulting ferrous alloy could not be forged between 90 940°-1010° C., and with 0.5% copper the alloy could not be forged between 890°-950° C., while with 0.75% copper the alloy could not be forged between 850°-910° C. This "red-shortness," or non-forgeability at red 95 heats, of copper-iron alloys means that these alloys cannot be satisfactorily worked or forged in a hot state. The presence of manganese or chromium in such quantity as we contemplate for improving the rust-resisting 100 properties of iron, eliminates this non-forging temperature range, so that the manganese- (or chromium) copper-iron alloy can be worked at all temperatures. The manganese or chromium, therefore, has the further function of rendering the ferrous alloy 105 malleable as well as of increasing its resistance to atmospheric corrosion, which function is of great importance in the practical use of the alloy. 110

While we have thus found that manganese of chromium added to a copper-iron alloy besides reducing the corrodibility, also enables the alloy to be forged without breaking, we have further determined that the 115 forging of the alloy becomes more difficult if the manganese or chromium content exceeds about 2%. Thus, copper-iron alloys containing over 2% of manganese or chromium are quite hard when hot and while such 120 alloys can be forged without breaking much more work is required in the forging operation. This means, of course, that in a steel mill a larger amount of work is required to produce sheets or bars from an alloy containing more than 2% of manganese or chromium than from an alloy containing less than 2% of manganese or chromium. The same general rule seems to hold with respect to grinding, filing and bending. With a 125 130

manganese or chromium content of less than 2% the alloy files and grinds easily and bends readily. With a manganese content greater than 2%, the alloy is difficult to 5 grind, is almost impossible to scratch with an ordinary file, and is quite brittle, while with a chromium content above about 2%, the alloy becomes tough and harder to work. These properties, within the range of copper 10 content contemplated by the present invention, appear to be a function of the manganese or chromium content and to be independent of the copper. For these reasons we deem it advisable in the practice of 15 our present invention, to use less than 2% of manganese or chromium, in combination with copper, for improving the rust-resisting properties of iron.

While our present invention is applicable 20 in principle to iron in any of its well known commercial forms, it is particularly applicable to steel and ingot iron because of the ease with which the metallic modifying agents can be added thereto. Thus, the copper 25 may be introduced by using pig or cast iron containing the necessary percentage of this metal, or pure copper or a suitable alloy of copper may be added to the molten iron, either in the furnace, in the ladle, or in the 30 molten ingot. The manganese may be added in the furnace or in the ladle as such or in the form of an alloy, such, for example, as ferro-manganese. Chromium may be introduced in substantially the same way as manganese 35 or by using a pig iron containing it. Further, steel scrap containing one or all of the metallic modifying agents may be used. The essential thing in any case is to get the modifying agents into the iron so 40 that they are uniformly distributed.

The matter of costs is of considerable importance in the case of iron or steel for ordinary commercial uses. It is, therefore, important to keep the cost of our improved 45 rust-resisting ferrous alloy as near as possible to the cost of ordinary iron or steel of a corresponding grade. The increased cost of our improved product above ordinary iron or steel of the same grade is due to 50 the required additions of the metallic modifying agents. As far as possible, therefore, we prefer to use scrap products for the introduction of such additional quantities of the modifying agents as our invention contemplates, and also, where possible, to use 55 materials in the production of the crude or unmodified iron or steel product which contain one or more of the modifying agents in quantities of value in the carrying out of 60 our invention.

Thus, instead of adding copper to the crude iron or steel, it is possible to use an iron ore containing copper, in which case the copper enters the iron or steel in the pig iron obtained in the blast furnace opera-

tion. The use of copper-bearing ores probably would not furnish all of the required amount of copper, so that additional amounts would have to be added to the molten iron. Such additions of copper may be obtained 70 from scrap products containing copper, such, for example, as turnings of German silver, Monel metal and the like. Where such copper alloys are employed it will be evident that metals other than copper may be introduced into the iron, but the quantities in which such other metals are present in the resulting ferrous alloy are relatively small and do not interfere with the effect of the copper or appreciably alter the properties 75 of the ferrous alloy.

In the smelting of iron ore for the production of pig iron, which later by remelting is changed to cast iron, or by remelting and refining becomes wrought iron, ingot 85 iron or steel, certain impurities in the ore itself, the coke and the slag, alloy with the iron. The most common of these impurities are carbon, phosphorus, sulfur, silicon and manganese, since these always occur in the 90 raw materials. In certain iron ores other elements exist and these also appear in the pig iron, such as copper, nickel, chromium and titanium. At the present time, manganese is almost universally used as a de-oxidizer of iron, and hence practically all commercial steels contain this element. In the refining process some of the impurities are oxidized in preference to the iron and are removed, while with others, the iron is 95 more readily oxidized and hence these latter are not removed but appear in the final product. To the former class belong carbon, silicon, phosphorus, sulfur, and manganese, while to the latter class belong copper and nickel. Chromium may be eliminated or not, as desired, depending upon the method used in refining. It may be said then that commercial irons and steels are 100 in an unstable state as regards corrosion and by the application of our present invention a great improvement can be effected in their 110 rust-resisting properties by small changes in the copper-manganese or copper-chromium, or copper-manganese-chromium content thereof.

Thus, by using ores, containing one or more of the metallic modifying agents contemplated by our present invention, the cost of making the additions of these agents to 120 the iron is much reduced. Iron ores containing copper, nickel and chromium, or chromium and nickel, may accordingly be advantageously used in the production of our improved rust-resisting ferrous alloy. 125 Take, for example, an iron ore containing 1 to 2% of chromium and 1% of nickel. In the smelting and refining of such an ore the nickel will appear in the iron while the chromium will or will not, depending upon 130

the process used. Here then, there exists a raw material, in the shape of the ore, which when used will give an alloy containing chromium and nickel to which copper must be added to produce a rust-resisting iron, and to which manganese will probably have to be added as a deoxidizer. This leads to a rather complex ferrous alloy containing chromium, manganese, copper and nickel. 5 The nickel is not added intentionally but gets into the final product since it exists in the ore. It will, therefore, be seen that our improved rust-resisting ferrous alloy may contain other metals besides the particular 10 modifying elements which we have found to exercise, in combination, such a beneficial effect upon the rust-resisting properties of iron. Such other metals are not intentionally introduced, but their presence is due to 15 the raw materials used in carrying out our invention. Although we prefer to use manganese or chromium, or both, as the minor modifying agent, any metal exercising in combination with copper the same effect in 20 improving the rust-resisting properties of iron may be used if desired. Thus tungsten, molybdenum, titanium and aluminum might be used instead of manganese or chromium, and in the appended claims we have designated 25 the minor modifying agents contemplated in the practice of the present invention as malleabilizing agents with respect to the influence of the copper on the malleability of the ferrous alloy, since, as previously 30 explained, the minor modifying agents serve to render malleable the ferrous alloy which would be otherwise non-malleable as a result of the copper present. It will, of course, be understood that by ferrous 35 alloy we mean an alloy containing principally iron and generally speaking we may say that our improved ferrous alloy contains at least 90% of iron.

We claim:

- 45 1. The improvement in the art of producing corrosion-resisting ferrous alloys which comprises ameliorating the normal tendency to corrode of an article composed principally of iron by associating with the 50 article in the form of an alloy with the iron a plurality of metallic modifying agents one of which is copper in excess of 0.5% and the other or others are malleabilizing agents with respect to the influence of the copper 55 on the malleability of the ferrous alloy, the combined effect of said modifying agents in ameliorating the corrosion-resisting properties of iron being more pronounced than is the effect of any one of the modifying 60 agents when used alone; substantially as described.
2. The improvement in the art of producing corrosion-resisting ferrous alloys which comprises ameliorating the normal tendency 65 to corrode of an article composed principally

of iron by associating with the article in the form of an alloy with the iron, a combined percentage of from about 1.5 to about 4 of a plurality of metallic modifying agents whose combined effect in improving the corrosion-resisting properties of iron is more pronounced than is the effect of any one of the modifying agents when used alone, one of said agents being copper and the other or others of said agents being malleabilizing 70 agents with respect to the influence of the copper on the malleability of the ferrous alloy; the amount of each agent present being from about 0.5% to 2%; substantially as described. 80

3. The improvement in the art of producing corrosion-resisting ferrous alloys which comprises ameliorating the normal tendency to corrode of an article composed principally of iron by associating with the article 85 in the form of an alloy with the iron a combined percentage of from about 1.5 to about 4 of copper and manganese, the copper and manganese being each present in an amount from about 0.5% to 2%; substantially as described. 90

4. The improvement in the art of producing corrosion-resisting ferrous alloys which comprises ameliorating the normal tendency to corrode of an article composed 95 principally of iron by associating with the article in the form of an alloy with the iron from about 1% to about 2% of copper and about 1% of manganese; substantially as described. 100

5. As a new article of manufacture, a corrosion-resisting ferrous alloy composed principally of iron and in which the normal tendency of the iron to corrode is ameliorated by the combined influence of from about 105 0.5% to about 2% of copper and from about 0.5% to about 2% of manganese associated in the form of an alloy with iron; substantially as described.

6. As a new article of manufacture, a corrosion-resisting ferrous alloy composed principally of iron and in which the normal tendency of the iron to corrode is ameliorated by the combined influence of such a percentage of copper as to render the ferrous 110 alloy when hot substantially non-malleable if alone contained therein and another metal whose effect in combination with the copper is to render the ferrous alloy malleable, said two metals operating together to produce a 115 more pronounced improvement in the corrosion-resisting properties of the ferrous alloy than would be produced by the use of either metal alone; substantially as described. 120

7. As a new article of manufacture, a corrosion-resisting ferrous alloy composed principally of iron and in which the normal tendency of the iron to corrode is ameliorated by the combined influence of from about 1% to about 2% of copper and such a 125 130

percentage of manganese as to render the resulting ferrous alloy malleable; substantially as described.

8. As a new article of manufacture, a corrosion-resisting ferrous alloy composed principally of iron and in which the normal tendency of the iron to corrode is ameliorated by the combined influence of such a percentage of copper as to render the ferrous alloy when hot substantially non-malleable if alone contained therein and such a percentage of manganese as to render the resulting ferrous alloy malleable; substantially as described.

15 9. As a new article of manufacture, a corrosion-resisting ferrous alloy composed principally of iron and in which the normal tendency of the iron to corrode is ameliorated by the combined influence of such a percentage of copper as to render the ferrous alloy when hot substantially non-malleable if alone contained therein and about 1% of manganese, substantially as described.

10. As a new article of manufacture, a corrosion-resisting ferrous alloy composed principally of iron and in which the normal tendency of the iron to corrode is ameliorated by the combined influence of from about 1% to 2% of copper and about 1% of manganese; substantially as described.

11. An article of manufacture which is subjected to corrosive influences comprising a ferrous alloy composed principally of iron and in which the normal tendency of the

iron to corrode is ameliorated by the combined influence of such a percentage of copper as to render the ferrous alloy when hot substantially non-malleable if alone contained therein, and another metal whose effect in combination with the copper is to render the ferrous alloy malleable, said two metals operating together to produce a more pronounced improvement in the corrosion-resisting properties of the ferrous alloy than would be produced by the use of either metal alone; substantially as described.

12. An article of manufacture which is subjected to corrosive influences comprising a ferrous alloy composed principally of iron and in which the normal tendency of the iron to corrode is ameliorated by the combined influence of from about 0.5% to about 2% of copper and from about 0.5% to about 2% of manganese associated in the form of an alloy with the iron; substantially as described.

13. An article of manufacture which is subjected to corrosive influences comprising a ferrous alloy composed principally of iron and in which the normal tendency of the iron to corrode is ameliorated by the combined influence of from about 1% to about 2% of copper and about 1% of manganese; substantially as described.

In witness whereof, we affix our signatures.

LINWOOD T. RICHARDSON.  
ELWOOD A. RICHARDSON.